

J. D. GALLAGHER.

BRAKE SHOE.

APPLICATION FILED MAY 27, 1911.

1,016,262.

Patented Feb. 6, 1912.



*Fig. 3.*



Attest:

*John Mitchell,  
R. N. Flint.*

by

Inventor:  
*Joseph D. Gallagher  
George C. Berk Atty*

# UNITED STATES PATENT OFFICE.

JOSEPH D. GALLAGHER, OF GLEN RIDGE, NEW JERSEY, ASSIGNOR TO EDWARD H. FALLOWS, TRUSTEE, OF NEW YORK, N. Y.

## BRAKE-SHOE.

1,016,262.

Specification of Letters Patent.

Patented Feb. 6, 1912.

Application filed May 27, 1911. Serial No. 629,792.

*To all whom it may concern:*

Be it known that I, JOSEPH D. GALLAGHER, a citizen of the United States, and a resident of Glen Ridge, in the county of 5 Essex and State of New Jersey, have made and invented certain new and useful Improvements in Brake-Shoes, of which the following is a specification.

My invention relates to an improvement in 10 brake shoes, and more particularly to that kind or type thereof comprising a cast metal body, and an insert embedded in the body, whereby to produce a compound wearing face, in order to secure the wearing or lasting 15 qualities, and at the same time the frictional or braking qualities in the shoe.

The object of my invention is to produce 20 such a shoe wherein the body will be made of cast iron, but of a much harder grade than heretofore used, and an insert, formed from wrought iron, or mild steel; such a shoe, I have found, by experiment, having a much 25 greater length of life in service than shoes of this type as heretofore made, and at the same time possessing all the necessary frictional or braking qualities.

With these and other ends in view, the invention consists in certain novel features of construction, as will be hereinafter fully 30 described and specifically pointed out in the claims.

In the accompanying drawing, Figure 1 is a view partly in side elevation, and partly broken away to show the wrought metal insert. Fig. 2 is a bottom plan view of the shoe, showing the wearing surface thereof. Fig. 3 is a view showing a section upon a transverse plane, indicated by the lines 3—3, of Fig. 1.

Referring to the drawings, 5 represents 40 the body portion of the shoe, and 6 the insert embedded therein, the former being made of cast metal, and the latter from mild steel or wrought iron; the insert may be of 45 any desired form or shape, but preferably that of a bar or ribbon bent or doubled upon itself to form a plurality of segments or parts extending longitudinally of the shoe, and arranged edgewise with reference to the 50 wearing face thereof. This insert may be provided with a series of holes 7, through which the cast metal of the body flows as the metal is poured, to thereby secure a better

anchorage or union between the insert and body.

The metal body portion 5 is formed from 55 hard cast metal, as, for example, from cast iron having a high percentage of sulfur and silicon to impart thereto a greater degree of hardness than is usually the case in brake 60 shoes of this character. The percentage of sulfur and of silicon employed may be varied considerably, depending largely upon the degree of hardness which it is desired to impart to the shoe. In practice, however, 65 I have found that about .40% of sulfur, and about 1.75% of silicon will produce satisfactory results. In the production of my improved brake shoe, the wrought metal insert is first properly bent or formed, and then 70 placed in the mold in which the body portion of the shoe is to be cast, after which the fluid metal is poured into the mold, and the insert thus embedded and securely anchored 75 in the body portion, the wrought metal insert serving not only to impart the necessary frictional qualities to the shoe, but also serving to hold the parts or sections of the shoe together, should it become cracked or 80 broken in service.

In brake shoes of the type described, and 85 having a wrought metal insert embedded in the cast metal body portion, the latter has commonly been formed from gray iron, and of a much softer grade as compared with the metal of which I form my improved shoe, the result being that in the old type the shoe wears away much more rapidly in service than in the case of my improved shoe. By 90 using, however, an insert of wrought iron or mild steel, the necessary frictional qualities are imparted to the shoe, these qualities, that is, the frictional and wearing qualities, combined in one shoe, producing an article much more economical and effective than 95 any shoe which has heretofore been produced.

I am aware that it is not new to construct 100 a brake shoe comprising a body of cast iron, and an insert of steel or wrought iron embedded therein, but I am not aware that any shoe has heretofore been made wherein the body has been formed from cast iron containing a high percentage of sulfur and silicon to impart thereto a great degree of 105 hardness, and wherein an insert has been

combined therewith formed from mild steel or wrought iron, and therefore:—

What I claim is:—

1. A brake shoe comprising a body portion formed from cast iron containing sulfur and silicon in sufficient quantities to impart hardness to said body portion in excess of the hardness possessed by cast iron alone; and an insert in the form of a ribbon 5 formed from a relatively soft metal, and bent to provide a plurality of segments, said ribbon being embedded in said body portion.
2. A brake shoe comprising a body portion formed from cast iron containing about 10 4% of sulfur, and about 1.75% of silicon; and an insert in the form of a ribbon formed from wrought iron and bent to provide a plurality of segments, said ribbon being embedded in said body portion.
3. A brake shoe comprising a body portion formed from cast iron containing quantities of sulfur and silicon sufficient to impart hardness to said body portion in excess 15 of the hardness of cast iron in which said

substances are absent, said body portion having an insert formed from wrought metal embedded therein.

4. A brake shoe comprising a body portion formed from cast iron containing sulfur and silicon in sufficient quantities to impart 20 hardness to said body portion in excess of the hardness possessed by cast iron alone, and an insert formed from a relatively soft metal and embedded in said body portion.

5. A brake shoe comprising a body portion formed from cast iron containing about 4% of sulfur, and about 1.75% of silicon, and an insert formed from wrought iron 25 embedded in said body portion.

Signed at New York, borough of Manhattan, in the county of New York and State of New York, this 25th, day of May, 40 A. D. 1911.

JOSEPH D. GALLAGHER.

Witnesses:

H. M. WHITE,  
A. V. WALSH.